# EUROPEAN PATENT SPECIFICATION

(11) **EP 0 179 212 B1**
(45) Date of publication and mention of the grant of the patent: **27.12.1991**
(21) Application number: 85109921.8
(22) Date of filing: 07.08.1985
(51) Int. Cl.: C23C 18/40

(54) **Chemical copper plating solution**
Stromlose Kupferplattierlösung
Bain de dépôt chimique de cuivre

(30) Priority: 27.09.1984 JP 200445/84; 26.12.1984 JP 273303/84
(43) Date of publication of application: 30.04.1986
(73) Proprietor: KABUSHIKI KAISHA TOSHIBA, Kawasaki-shi, Kanagawa-ken 210 (JP)
(72) Inventor: Endo, Akira, Saiwai-ku Kawasaki-shi Kanagawa-ken (JP); Takeda, Kazuhiro, Saiwai-ku Kawasaki-shi Kanagawa-ken (JP)
(74) Representative: Lehn, Werner, Dipl.-Ing.

(56) References cited:
- EP-A- 0 039 757
- EP-A- 0 107 087
- FR-A- 2 436 192
- US-A- 3 377 174
- US-A- 3 661 597
- US-A- 3 902 907
- US-A- 3 959 531

## Description

This invention relates to a chemical copper plating solution. More particularly, it is concerned with a chemical copper plating solution having a novel composition which makes it possible to deposit copper at a high speed and is stable over a prolonged period of application and can form a plated film having favourable mechanical properties.

A chemical copper plating solution may usually contain as essential components a water-soluble copper salt such as copper sulfate, cupric chloride, etc.; a complexing agent such as ethylenediaminetetraacetic acid (EDTA), N,N,N',N'-tetrakis-(2-hydroxypropyl)ethylenediamine, Rochelle salt, etc.; a reducing agent such as formaldehyde, dimethylaminoborane, sodium borohydride, etc.; a pH adjustor such as sodium hydroxide, potassium hydroxide, etc.; and, where necessary, a surface active agent such as a polyethylene oxide, a polyether, a polyester, etc.

However, a chemical copper plating solution having the composition of such components generally tends to lack stability and readily undergo self-decomposition; moreover, a plated film or deposited film made from said chemical plating solution is brittle and insufficient in mechanical strength, particularly bending strength for practical utility.

In order to improve such defects, there has been proposed a chemical copper plating solution wherein there were further added a variety of additives, e.g., a dipyridyl, a phenanthroline, a water-soluble cyan compound, an inorganic or organic sulfur compound or a polymeric substance, in addition to prior plating components, i.e., a copper salt, a complexing salt, a reducing agent and a pH adjustor (see Japanese Patent Publications Nos. 1084/1965 and 11521/1968 and Japanese Provisional Patent Publication No. 68033/1977.).

EP-A-0 039 757 discloses a chemical copper-plating solution capable of providing a plated film, excellent especially in ductility. The solution comprises a copper salt, a complex-forming agent, a reducing agent and a pH-controller and a nonionic surfactant having the formula
wherein m and n are integers of 1 or more, and wherein m + n ≧ 12. This solution may further contain at least one compound selected from the group consisting of 1,10-phenanthroline, 1,10-phenanthroline derivatives, 2,2'-dipyridyl, 2,2'-biquinoline and water-soluble cyanides.

However, even when the above-mentioned components would be added, stability of a plating solution and mechanical properties of a plated film have not yet been improved satisfactorily and, further, there have been inevitably presented problems of a slower deposit rate in plating and a reduced productivity owing to such components supplemented.

### SUMMARY OF THE INVENTION

The primary object of this invention is to provide a chemical copper plating solution having a novel composition which can dissolve the aforesaid problems, show a good stability, without reducing high speed deposit in plating, and provide good mechanical properties, especially a favourable spreadability of the resultant plated film.

The chemical copper plating solution of this invention is a chemical copper plating solution containing a copper salt, a complexing agent, a reducing agent and a pH adjustor, which further comprises the under-mentioned Group:
(A) at least one nonionic surface active agent selected from the group consisting or a non-ionic surface active agent having the formula (I): (wherein m₁ and n₁ each represent an integer of 1 or more); and
   a nonionic surface active agent having the formula (II): (wherein m₂ and n₂ each represent an integer of 1 or more);
   and at least one selected from the group consisting of 1,10-phenanthroline, a 1,10-phenanthroline derivative, 2,2'-dipyridyl, 2,2'-biquinoline and a water-soluble cyan compound.

In a specific embodiment of the invention the chemical copper plating solution may furthermore contain the following group (B):
(B) an organic sulfur compound and/or an ethyleneamine compound.

### DESCRIPTION OF THE PREFERRED EMBODIMENTS

The chemical copper plating solution according to this invention is composed of, in addition to the four components of a copper salt, a complexing agent, a reducing agent and a pH adjustor, compounds of the group (A) comprising (i) at least one compound selected from the group consisting of nonionic surface active agents mentioned below and (ii) at least one Compound selected from the group consisting of 1,10-phenanthroline, a 1,10-phenanthroline derivative, 2,2'-dipyridyl, 2,2'-biquinoline and a water-soluble cyan compound; favourably the composition furthermore comprises as group (B) an organic sulfur compound and/or an ethyleneamine compound.

Of these components, a copper salt may supply a copper ion, while a reducing agent may reduce said copper ion to a metallic state. A complexing agent may form a stable complex with copper ions to prevent, in a plating bath (alkaline), a formation of cupric hydroxide, while a pH adjustor may adjust the optimum plating deposit potential in a plating bath. These components may be of any of those usually employed for the preparation of a prior chemical copper plating solution.

Of the Group (A), the nonionic surface active agent may contribute to mechanical properties and deposit rate of a plating solution and is represented by the formula (I) or (II).

In the formulae (I) and (II), each of m₁, m₂, n₁ and n₂ is an integer of 1 or more. If any of them is 0 (zero), a nonionic surface active agent shows a low solubility so that a sufficient amount thereof to contribute to improvement in stability or mechanical properties of a plating solution could not be dissolved in a plating solution. On the other hand, as m₁ + n₁ or m₂ + n₂ is increased, stability and mechanical properties of a plating solution may be correspondingly improved. In any case, its effect may approximately reach the upper limit at the neighborhood of 20 to a saturated state. Thus, here is particularly no upper limit with regard to m₁ + n₁ or m₂ + n₂, but not more than 500 is preferred in view of workability.

A concentration of the compound (I) or (II) in a plating solution is preferably in the range of 10 mg/l to 30 g/l. In particular, where each of m₁ + n₁ and m₂ + n₂ is less than 20, a range of 30 mg/l to 20 g/l is preferred. Where each of m₁ + n₁ and m₂ + n₂ is not less than 20, a range of 10 mg/l to 5 g/l is preferred.

In this invention, there is further added at least one of 1,10-phenanthroline, a 1,10-phenanthroline derivative, 2,2'-dipyridyl, 2,2'-biquinoline or a water-soluble cyan compound, in order that the aforesaid effects by nonionic surface active ageant, especially stability of a plating solution or mechanical properties of a plated film may be far more enhanced.

The 1,10-phenanthroline derivative may preferably have a substituent such as a lower alkyl group, e.g., a methyl group, an ethyl group, etc. or a phenyl group and there may illustratively be mentioned 2,9-dimethyl-1,10-phenanthroline, 4,7-diphenyl-2,9-dimethyl-1,10-phenanthroline, 4,7-diphenyl-1,10-phenanthroline and so on.

As the water-soluble cyan compound, there may be mentioned, for instance, potassium cyanide, sodium cyanide, sodium nitroprusside, potassium ferrocyanide, potassium ferricyanide, potassium tetracyanoniccolate and so on.

A total amount of 1,10-phenanthroline, a 1,10-phenanthroline derivative, 2,2'-dipyridyl and 2,2'-biquinoline to be added is preferably 1 - 200 mg/l, a range of 2 - 50 mg/l being particularly preferred. If the added amount is less than 1 mg/l, one could not obtain effects at all; if said amount is more than 200 mg/l, there would undesirably produce a reduced stability of a plating solution or a reduced mechanical property of a plated film.

An amount of the water-soluble cyan compound to be added is preferably 1 mg/l to 3 g/l, a range of 5 mg/l to 1 g/l being particularly preferred. If the added amount is less than 1 mg/l, it does not at all contribute to improvement in stability and mechanical properties, while, if more than 3 g/l, there would undesirably produce a lowered deposit rate or a reduced mechanical property of a plated film.

Also, the organic sulfur compound added as the Group (B) may contribute to improved stability of a plating solution, while the ethyleneamine compound may contribute to speed-up of a deposit rate.

As the organic sulfur compound which may be employed as the Group (B), there may be mentioned, for instance, 2-mercaptobenzothiazole, thiourea, ethylene thiourea, 1-phenyl-2-thiourea, 1-allyl-2-thiourea, thiodiglycol, thiomalic acid, thiodiethanol, 2-mercaptobenzimidazole, dodecylmercaptan, thioglycolic acid, thiodiglycolic acid, etc. An amount of the organic sulfur compound to be added is preferably 0.01 mg/l to 10 mg/l, a range of 0.1 mg/l to 5 mg/l being particularly preferred. If the added amount is less than 0.01 mg/l, stability of a plating solution is not so much improved; if more than 10 mg/l, a deposit rate is extremely lowered, which leads to a reduced working efficiency.

As the ethyleneamine compound, there may be mentioned, for instance, ethylenediamine, diethylenetriamine, triethylenetetramine, tetraethylenepentamine, pentaethylenehexamine and so on. An amount of the compound to be added is preferably 1 mg/l to 500 mg/l, a range of 5 mg/l to 100 mg/l being particularly preferred. If the added amount is less than 1 mg/1, a deposit rate of the plating solution or mechanical properties of the plated film is not so much improved; if more than 500 mg/l, a plating solution becomes unstable.

The chemical copper plating solution of the present invention can become a chemical copper plating solution having respective merits of the compounds, that is to say, the plating solution having an excellent stability and producing a highly spreadable plated film with a high speed deposit, when the above compounds having the above-mentioned functions are used in combination therewith at the predetermined proportion.

Preferable plating conditions, under which the present chemical copper plating solution may be applied, are the range of a temperature of 40 - 80 ^{o}C, more preferably 50 - 70 ^{o}C and a pH value of 10.8 - 13.0, more preferably 12.0 - 13.0. According to such plating condition, characteristic of the present plating solution can be fully put to use and there can be formed a plated film which can be deposited at a high speed and has a high spreadability.

This invention will be more fully illustrated by way of the following examples.

### Examples 1 - 12

A stainless steel plate with a thickness of 0.3 mm was polished with a cleanser, dipped in a 10 % sodium hydroxide solution at 80 ^{o}C for one minute, taken out and washed with water. Then, it was dipped in a 10 % sulfuric acid at ordinary temperature for 30 seconds and washed with water to clean the surface thereof. The resultant stainless steel plate was then dipped in a solution having the composition of;

for 2 minutes and washed in a running water for one minute. Thereafter, the plate was dipped in a solution having the composition of;

for one minutes and washed in a running water for one minute.

On the other hand, there were prepared various chemical copper plating solutions having the following compositions;

The chemical copper plating solutions thus prepared were measured for deposit rate of copper. Such a measurement was accomplished by dipping a copper foil with a thickness of 10 µm, the surface of which was previously cleaned, in the plating solution under conditions of a plating temperature of 60 ^{o}C and a pH value of the plating solution of 12.5 for one hour and calculating a deposit rate from the difference in weight before and after plating.

Then, the catalyzed stainless steel plate with a thickness of 0.3 mm as described above was treated with the chemical cooper plating solution to deposit plated films with a thickness of 30 - 35 µm over both sides thereof, respectively, using plating conditions of a plating temperature of 60 ^{o}C and a pH value of the plating solution of 12.5.

The copper plated film thus deposited was peeled off from the stainless steel plate and applied to a spreadability test. Spreadability was measured according to the following folding test at 180 ^{o}C; a plated film was first folded to one direction at 180 ^{o} to make a fold and then restored to an original position and pressed to flat the fold. Such a procedure was counted as one folding and repeated until the plated film was broken at the folding portion. According to this test, spreadability of the plated film is represented in terms of the numbers of foldings which the plated film could resist.

Also, stability of the plating solution was evaluated by repeating dipping of the material to be plated, while properly supplementing a plating bath with components of respective plating compositions, counting as one cycle the point when all copper ions originally involved were deposited and measuring how many cycles the plating solution would be not usable by self-decomposition.

The results are summarized in Table 1, with regard to corresponding copper plating solutions, wherein deposit rate (µm/hr) of each copper plated film is also shown. The numbers of 1 - 12 in Table 1 indicate the Examples of the present invention.

And nonionic surface active agents of the formulae (I) and (II) are represented with A-x and B-x, respectively, said "x"s in A-x and B-x indicating m₁ + n₁ and m₂ + n₂, respectively.

### Comparative Examples 1 - 2

In Comparative Example 1, a plating solution was prepared in the same manner as in the above Examples except for using a compound other than the present invention in place of the component other than the nonionic surface active agents in the Group(A).

While a plating solution for Comparative Example 2 was prepared in the same manner as in the above Examples except for using a compound other than the present invention in place of the nonionic surface active agent in the Group (A).

Then, similar tests as in the above Examples were carried out to those and the results are also shown in Table 1.

As explained hereinabove, the chemical copper plating solution of the present invention can show an excellent stability usable over prolonged period, together with a high speed deposit, and produce a plated film having superior mechanical properties, inter alia, a good spreadability as illustrated with folding strength.

Accordingly, application of the chemical copper plating solution of the present invention can greatly improve working efficiency for plating and further enhance reliability in forming a plated film.

Therefore, the chemical copper plating solution of the present invention may be most suitable for production of, e.g., a continuity circuit in a print distributing plate and is highly valuable in an industrial field.

## Claims

1. A chemical copper plating solution containing a copper salt, a complexing agent, a reducing agent and a pH adjustor which further comprises the following Group (A):
Group (A):
at least one nonionic surface active agent selected from the group consisting of a nonionic surface active agent having the formula: (wherein m₁ and n₁ each represent an integer of 1 or more) and a non-ionic surface active agent having the formula: (wherein m₂ and n₂ each represent an integer of 1 or more);
and at least one compound selected from the group consisting of 1,10-phenanthroline, a 1,10-phenanthroline derivative, 2,2'-dipyridyl, 2,2'-biquinoline and a water-soluble cyan compound.

2. A chemical copper plating solution as claimed in claim 1, which furthermore comprises the following Group (B):
Group (B);
an organic sulfur compound and/or an ethyleneamine compound.

3. The chemical copper plating solution as claimed in Claim 1 or 2,wherein the complexing agent is a cupric ion complexing agent.

4. The chemical copper plating solution as claimed in Claim 2, wherein the ethyleneamine compound is an ethylenepolyamine compound.

5. The chemical copper plating solution as claimed in Claim 1 or 2, wherein a concentration of the nonionic surface active agent of the formula (I) and (II) is 10 mg/l to 30 g/l.

6. The chemical copper plating solution as claimed in Claim 1 or 2, wherein the m₁ + n₁ and m₂ + n₂ are each not more than 500.

7. The chemical copper plating solution as claimed in Claim 1 or 2, wherein a total concentration of 1,10-phenanthroline, a 1,10-phenanthroline derivative, 2,2'-dipyridyl and 2,2'-biquinoline is 1 - 200 mg/l.

8. The chemical copper plating solution as claimed in Claim 1 or 2, wherein a concentration of the water-soluble cyan compound is 1 mg/l to 3 g/l.

9. The chemical copper plating solution as claimed in Claim 2, wherein a concentration of the organic sulfur compound is 0.01 - 10 mg/l.

10. The chemical copper plating solution as claimed in Claim 2, wherein a concentration of the ethyleneamine compound is 1 - 500 mg/l.

11. A method for application of a chemical copper plating solution as claimed in Claim 1 or 2, wherein application condition is 40 - 80 ^{o}C and pH of 10.8 - 13.0.

## Revendications

1. Solution de cuivrage chimique contenant un sel de cuivre, un agent complexant, un agent réducteur et un agent d'ajustement du pH qui comprend en outre le Groupe (A) suivant :
Groupe (A) :
- au moins un agent tensio-actif non ionique choisi parmi le group consistant d'agent tensio-actif non-ionique répondant à la formula : (dans laquelle m₁ et n₁ représentent chacun un entier égal à 1 ou davantage) et un agent tensio-actif non ionique répondant à la formule : (dans laquelle m₂ et n₂ représentent chacun un entier égal à 1 ou davantage);
et au moins un composé choisi parmi le group consistant de la 1,10-phénanthroline, un dérivé de la 1,10-phénanthroline, le 2,2'-dipyridyle, la 2,2'-biquinoléine et un composé cyané soluble dans l'eau.

2. Solution de cuivrage chimique selon la revendication 1, qui comprend en outre le Groupe (B) suivant :
Groupe (B) :
- un composé soufré organique et/ou une éthylèneamine.

3. Solution de cuivrage chimique selon les revendications 1 ou 2, dans laquelle l'agent complexant est un agent complexant de l'ion cuivrique.

4. Solution de cuivrage chimique selon la revendication 2, dans laquelle l'éthylèneamine est une éthylène polyamine.

5. Solution de cuivrage chimique selon les revendications 1 ou 2, dans laquelle la concentration de l'agent tensio-actif non ionique répondant aux formules (I) et (II) est de 10 mg/l à 30 g/l.

6. Solution de cuivrage chimique selon les revendications 1 ou 2, dans laquelle m₁ + n₁ et m₂ + n₂ sont chacun non supérieurs à 500.

7. Solution de cuivrage chimique selon les revendications 1 ou 2, dans laquelle la concentration totale de la 1,10-phénanthroline, du dérivé de la 1,10-phénanthroline, du 2,2'-dipyridyle, et de la 2,2'-biquinoléine est de 1 à 200 mg/l.

8. Solution de cuivrage chimique selon les revendications 1 ou 2, dans laquelle la concentration du composé cyané soluble dans l'eau est de 1 mg/l à 3 g/l.

9. Solution de cuivrage chimique selon la revendication 2, dans laquelle la concentration du composé soufré organique est de 0,01 à 10 mg/l.

10. Solution de cuivrage chimique selon la revendication 2, dans laquelle la concentration de l'éthylèneamine est de 1 à 500 mg/l.

11. Procédé d'utilisation d'une solution de cuivrage chimique selon les revendications 1 ou 2, dans lequel les conditions d'utilisation sont une température de 40 à 80^{o}C et un pH de 10,8 à 13,0.

## Patentansprüche

1. Chemische Kupferplattierlösung, umfassend ein Kupfersalz, ein Komplexierungsmittel, ein Reduktionsmittel und ein pH-Einstellmittel, welche weiterhin die folgende Gruppe (A) enthält
Gruppe (A):
zumindest ein nicht-ionisches oberflächenaktives Mittel, ausgewählt aus der Gruppe, bestehend aus einem nicht-ionischen, oberflächenaktiven Mittel der Formel (worin m₁ und n₁ jeweils eine ganze Zahl von 1 oder mehr bedeuten) und einen nicht-ionischen oberflächenaktiven Mittel der Formel (worin m₂ und n₂ jeweils eine ganze Zahl von 1 oder mehr darstellen);
und zumindest eine Verbindung, ausgewählt aus der Gruppe, die aus 1,10-Phenanthrolin, einem 1,10-Phenanthrolinderivt, 2,2'-Dipyridyl, 2,2'-Dichinolin und einer wasserlöslichen Cyanverbindung besteht.

2. Chemische Kupferplattierlösuung nach Anspruch 1, dadurch **gekennzeichnet**, dass sie weiterhin die folgende Gruppe (B) umfasst:
Gruppe (B):
eine organische Schwefelverbindung und/oder eine Ethylenaminverbindung.

3. Chemische Kupferplattierlösung nach Anspruch 1 oder 2, dadurch **gekennzeichnet**, dass das Komplexierungsmittel ein
Kupferionen-Komplexierungsmittel ist.

4. Chemische Kupferplattierlösung nach Anspruch 2, dadurch **gekennzeichnet**, dass die Ethylenaminverbindung eine Ethylenpolyaminverbindung ist.

5. Chemische Kupferplattierlösung nach Anspruch 1 oder 2, dadurch **gekennzeichnet**, dass eine Konzentration des nicht-ionischen oberflächenaktiven Mittels der Formel (I) und (II) 10 mg/l bis 30 g/l ausmacht.

6. Chemische Kupferplattierlösung nach Anspruch 1 oder 2, dadurch **gekennzeichnet**, dass m₁ + n₁ und m₂ + n₂ jeweils nicht mehr als 500 ausmachen.

7. Chemische Kupferplattierlösung nach Anspruch 1 oder 2, dadurch **gekennzeichnet**, dass eine Gesamtkonzentration von 1,10-Phenanthrolin, einem 1,10-Phenanthrolinderivat, 2,2'-Dipyridyl und 2,2-Dichinolin 1 bis 200 mg/l ausmacht.

8. Chemische Kupferplattierlösung nach Anspruch 1 oder 2, dadurch **gekennzeichnet,** dass eine Konzentration der wasserlöslichen Cyanverbindung 1 mg/l bis 3 g/l ausmacht.

9. Chemische Kupferplattierlösung nach Anspruch 2, dadurch **gekennzeichnet,** dass die Konzentration der organischen Schwefelverbindung 0,01 bis 10 mg/l ist.

10. Chemische Kupferplattierlösung nach Anspruch 2, dadurch **gekennzeichnet,** dass die Konzentration der Ethylenaminverbindung 1 bis 500 mg/l ist.

11. Verfahren zur Anwendung einer chemischen Kupferplattierlösung nach Anspruch 1 oder 2, dadurch **gekennzeichnet,** dass die Anwendungsbedingung 40 bis 80°C und der pH-Wert 10,8 bis 13,0 sind.
